

UNITED STATES PATENT OFFICE

2,387,501

## HYDROCARBON OIL

**Melvin A. Dietrich, Claymont, Del., assignor to  
E. I. du Pont de Nemours & Company, Wil-  
mington, Del., a corporation of Delaware**

**No Drawing. Application April 4, 1944,  
Serial No. 529,512**

14 Claims. (Cl. 252—47.5)

This invention relates to hydrocarbon oils and more particularly to hydrocarbon oil compositions having low pour points, high viscosity indexes and improved stability against breakdown under oxidizing conditions.

Hydrocarbon oils, derived from paraffin and mixed base crude oils, contain considerable amounts of paraffin wax which causes the oil to become solid at low temperatures and, in the case of lubricating oils, prevents a quick and effective flow of the lubricant to moving parts. Such wax may be removed from the oil by cold settling or by dilution with low boiling naphtha followed by chilling and centrifuging or filtration. These processes are expensive and may, if complete removal of the wax is effected, result in lubricants with reduced viscosity indexes. In the low viscosity mineral oils, such as those boiling above the kerosene range and which are used as fuels in compression-ignition engines, the presence of wax may result in congelation of the oil in storage tanks at low temperatures. Complete removal of the wax may result in a fuel with unsatisfactory combustion characteristics.

The change in the viscosity of oils, with variations in temperature, is well known. A high rate of change of viscosity with change in temperature is generally considered undesirable since, for many lubricant uses, it results in an oil with too low viscosity for use at high temperatures and too high viscosity for use at low temperatures. In the case of fuel oils, too rapid change of viscosity with change in temperature may result in unsatisfactory carburetion and poor combustion of the fuel.

Hydrocarbon oils, on being subjected to the action of heat, air and metals, tend to oxidize and form insoluble products which deposit in oil lines, heat exchangers, crankcases, storage tanks and the like. These deposits generally result in reduced flow of oil to the bearing surfaces and may shut off such flow altogether by clogging oil holes.

Many substances have been proposed for addition to hydrocarbon oils for the purpose of improving the properties of the oils in each of the above respects. Such substances include polymerized olefines, condensation products of aromatic hydrocarbons with chlorinated paraffin wax, mixed aryl alkyl ketones, and fatty acids and their salts and esters. These various substances have been found to act with varying degrees of efficiency in improving the properties of the oil with respect to one of the characteristics above discussed, but generally have no beneficial effect on other properties of the oil. This has generally made it necessary to add several different sub-

stances to an oil in order to obtain the desired effect on the different properties of the oil. This is objectionable and those skilled in the art have long searched for a single substance which will improve the pour point, the viscosity index and the stability of the oil against oxidative breakdown.

down.

It is an object of the present invention to provide a material for addition to hydrocarbon oils to improve the various properties of the oil. A particular object of my invention is to provide hydrocarbon oils with reduced pour points and improved flow characteristics at low temperatures. Another particular object of my invention is to provide a hydrocarbon oil with a low rate of change of viscosity with change in temperature, that is, with a high viscosity index. A further particular object of the present invention is to provide a hydrocarbon oil having a high resistance to oxidation and a reduced tendency to form insoluble products under oxidizing conditions. A still further object is to provide a hydrocarbon oil which is improved with respect to pour point, viscosity index and stability against oxidative breakdown.

25 My invention against oxidative breakdown.

The above and other objects may be accomplished in accordance with my invention which comprises incorporating in a hydrocarbon oil a small proportion of an oil-soluble polymeric N-  
30 aliphatic acrylamide having a molecular weight of at least 1000 in which the aliphatic group contains an open chain of at least 8 atoms of which not more than 2 are interrupting atoms of the group of oxygen and sulfur and the rest are carbon atoms. I have found that such polymeric acrylamides, when incorporated in a hydrocarbon oil, are very effective to reduce the pour point, increase the viscosity index and increase the stability of the oil against oxidative breakdown.  
35

40 Thus, by my invention, I am able to improve several properties of a hydrocarbon oil by the incorporation therein of a single substance.

The oil-soluble polymeric N-aliphatic acrylamides, which are to be employed in accordance with my invention, may be defined as polymers whose monomeric unit is considered to be



wherein each of R and R' represents a hydrogen atom or an aliphatic hydrocarbon group and R'' is an acyclic aliphatic group containing a chain of at least 8 atoms, not more than 2 of which atoms are interrupting atoms of oxygen or sulfur

and the rest of which atoms are carbon atoms. These compounds may be obtained by the reaction of the appropriate amine with an acrylic acid ester which may be monomeric or polymeric.

The acrylic acid esters, from which my compounds may be derived, may be represented by the formula



wherein R represents a hydrogen atom or an aliphatic hydrocarbon group and R''' represents an esterifying organic group. Preferably, R will represent hydrogen or a short-chain alkyl group, such as methyl, ethyl and propyl. Also preferably, R''' will be a short-chain alkyl group. Representative acrylic acid esters are the esters of acrylic acid, methacrylic acid, ethylacrylic acid and propylacrylic acid.

The amines, which may be employed in the preparation of the amides, which are to be employed in accordance with my invention, may be represented by the formula



wherein R' represents hydrogen or an aliphatic hydrocarbon group and R'' represents an aliphatic group which contains an open chain of at least 8 atoms, not more than 2 of such atoms being interrupting oxygen or sulfur atoms and the rest of such atoms being carbon atoms. The aliphatic chain, represented by R'', may be a straight chain or a branch chain and may be saturated or unsaturated. Generally, it will be preferred that R'' be a hydrocarbon group, that is, one which consists of carbon and hydrogen. However, the chain represented by R'' may be substituted by other elements or groups, such as halogens, nitro and divalent sulfur-containing and oxygen-containing groups, particularly in the form of ether or thioether linkages. Representative of such substituents are chlorine, fluorine, nitro, ethoxy, isobutoxy, benzylthio, benzyl, cyclohexyl, naphthyl and naphthylthio. Preferably, the amines will be primary amines, that is, those in which R' represents hydrogen. Primary amines, derived from vegetable, animal or fish oils or by the oxidation and amination of paraffin or other petroleum fractions, may be used. Amines, derived from hydrogenated coconut oil alcohols and naphthyl amines, are especially useful. By the term "alkyl" group, as employed herein, I mean a saturated aliphatic hydrocarbon group.

The polymeric N-aliphatic acrylamides, employed in accordance with my invention, may be prepared by the polymerization of monomeric acrylamides or by heating polymeric acrylic esters with the appropriate amine until substitution has taken place. Generally, more effective products are obtained by reacting the amine with the polymeric acrylic esters. The reactants will be mixed and heated together at temperatures sufficiently high to decompose the ester and drive off the esterifying alcohol. The temperature employed will be determined by the ease of the reaction and by the boiling point of the amine, but will generally be within the range of from about 125° C. to about 250° C. The time of reaction will generally be from about 1 to about 8 hours. It is not necessary to prepare the polymeric amides from a single ester and a single amine, but mixtures of esters

and mixtures of amines may be employed in the reaction.

The polymeric amides will vary from gummy materials, which can be pulled into threads and filaments, to soft rubbery materials and materials which resemble a soft tough glass at ordinary temperatures. They will have molecular weights which may vary from 1000 to as high as 50,000. Preferably, I employ polymers having a molecular weight of from about 5000 to about 25,000.

By a hydrocarbon "oil," I mean one which has a viscosity of at least 35 seconds Saybolt at 100° F., and intend to include therein oils in the fuel oil range, including Diesel fuels and furnace oils, as well as the higher viscosity oils, employed as lubricating oils and greases. The oils may be solvent extracted oils or conventionally refined oils, obtained from various base crude oils. They may be specially compounded oils, such as those containing lard oil, fish oil, castor oil or the like. When the oils are fuel oils, designed for use in high speed Diesel engines, they may contain ignition primers, such as ethyl nitrate. The polymeric materials may be added to refined oils or may be added to the oils during any suitable stage in the refining process. The use of the polymeric amides of my invention in fuel oils is of considerable importance since it permits the manufacture and use of fuel oils of higher paraffin content and improved ignition qualities.

The quantity of polymer to be added to the oil will vary within wide limits and will depend on the effect it is desired to produce. Thus, if pour point depressant action alone is desired, as little as 0.01% may suffice with the preferred range lying between 0.02% and about 1.0%. If improvement of viscosity index is the main consideration a larger amount of polymer will normally be required, the preferred quantity ranging from about 1.0% to about 5.0%. In fuel oils, preferred ranges of concentration lie between about 0.01% and about 5.0%. The products may be used in conjunction with other additives such as organic phosphates or phosphites, for example, tricresyl phosphate or tributyl phosphite; metal soaps or additives, for example, copper naphthenate, tin oleate, chromium oleate, or copper derivatives of terpene mercaptans; sulfur-containing stabilizers, such as sulfurized sperm oil, S-alkylated 2-mercaptothiazolines, and dialkylthiuram disulfides.

The products may be used in mineral oils for the preparation of greases. In this case, higher concentrations, than those mentioned heretofore, may be needed. Thus, concentration ranges of about 5.0% to about 50.0% may be needed to produce greases of satisfactory consistency. In the preparation of greases, the polymers may be used in conjunction with metal soaps such as sodium, calcium, lithium, aluminum, and barium naphthenates or stearates.

The polymeric amides of my invention may be employed in refining oils in conjunction with solvent dewaxing processes whereby a more efficient separation of wax occurs and a product of very low pour point is obtained. In the dewaxing of paraffin base oils, the distillate is mixed with a solvent naphtha, the mixture is chilled to about -20° F. and then filtered or centrifuged to remove the precipitated wax. This wax contains considerable amounts of absorbed oil which requires removal to obtain a high melting and commercially useful paraffin. The

addition of the polymeric amides of my invention to the solvent naphtha-oil mixture, prior to chilling, produces a wax which contains lesser amounts of absorbed oil than it would otherwise contain. This results in high yields of the dewaxed oils as well as a better wax. At the same time, the dewaxed oil thus obtained has its properties improved by the presence of the polymeric amide which is carried through the process with the oil.

In order to more clearly illustrate my invention, the preferred modes of carrying the same into effect and the advantageous results to be obtained thereby, the following examples are given in which the amounts are by weight, except where otherwise specifically indicated.

*Example I*

Three parts of monomeric octadecyl methacrylamide were melted on a steam bath, a trace of benzoyl peroxide added, and the mixture heated on the steam bath for three hours. This material at the end of this time was thick and viscous while hot. On cooling it resembled a soft, tough glass. When 0.5% by weight of the product was dissolved in an SAE 30 paraffin base oil, the pour point was lowered from 30° F. to 0° F. When 2.0% of the material was dissolved in a paraffin base distillate the following viscosity changes were noted:

|                                                | Original oil | Oil+2% polymer |
|------------------------------------------------|--------------|----------------|
| Saybolt Universal viscosity at 100° F. seconds | 322          | 406            |
| Saybolt Universal viscosity at 210° F. do      | 63           | 59.4           |
| Viscosity index                                | 92           | 102            |

The viscosity index noted above was calculated by the method of Dean and Davis described in Chem. and Met. Eng. 36, 618 (1929). This index serves as a measure of the flatness of the viscosity-temperature curve. With increasing values of the index, viscosity-temperature curves become flatter.

*Example II*

Ten parts of methyl methacrylate polymer and 27 parts of octadecylamine were mixed and heated to 250° C. for one hour. The reaction mass was dissolved in benzene, filtered, and evaporated in vacuo. The residue was a gummy gray material which could be pulled into threads and filaments and which weighed 33 parts. It contained 37.4% nitrogen. The effect of this material on pour point is shown as follows:

| Percent by weight of polymer in oil | Pour point of SAE 30 paraffin base oil, °F. |
|-------------------------------------|---------------------------------------------|
| 0                                   | 30                                          |
| 0.1                                 | -5                                          |
| 0.17                                | +5                                          |
| 0.27                                | 6                                           |
| 0.33                                | 0                                           |

A 2% solution in the paraffin base distillate given in Example I raised the viscosity index from 92 to 115. The characteristics of the treated oil were: viscosity at 100° F., 359 seconds; at 210° F., 59.1 seconds.

*Example III*

A second batch of product, prepared as described in Example II, was dissolved in a solvent-refined Mid-Continent SAE 30 oil to form a 0.5% solution by weight. This oil was then tested for

stability against formation of deposits by the method described in U. S. 2,236,168. The results obtained are as follows:

|                               | Deposit, mg/30 cc. oil |
|-------------------------------|------------------------|
| Untreated oil                 | 232                    |
| Treated oil                   | 163                    |
| Reduction in deposit per cent | 30                     |

*Example IV*

10 Twenty parts of polymeric methyl methacrylate and 53 parts of oleylamine were mixed and heated for 2 hours at 250° C. with stirring. The mass was cooled, dissolved in benzene, filtered, and evaporated in vacuo. Seventy parts of a soft rubbery polymer were obtained. A 2% solution of this product in an SAE 30 paraffin base oil yielded the following viscosity data:

|                                                | Original oil | Oil+2% polymer |
|------------------------------------------------|--------------|----------------|
| Saybolt Universal viscosity at 100° F. seconds | 323          | 358            |
| Saybolt Universal viscosity at 210° F. seconds | 52.4         | 57.4           |
| Viscosity index                                | 87           | 107            |

*Example V*

30 The stability of the product under service conditions was demonstrated by means of an engine test, using a 0.33% oil solution of the product, prepared as in Example II from octadecylamine and methyl methacrylate polymer. The oil had an initial pour point, prior to treatment with the polymer, of 25° F. After treatment to form a .033% solution, the pour point was -10° F. The oil solution was then operated in a Chevrolet engine for 36 hours at 2500 R. P. M. with an oil temperature of 250° F. and a jacket temperature of 160° F. At the end of this period the pour point of the oil was -5° F., substantially the same as the pour point at the start of the test.

35 It will be understood that the preceding examples are given for illustrative purposes only and that various modifications and variations may be made therein without departing from the spirit or scope of my invention, my invention not being limited to the specific embodiments disclosed, except as indicated in the following claims. For example, in addition to the substances employed in the examples, the following polymeric amides come within the scope of this invention:

- 55 N-octylpolymethacrylamide
- N-2-ethylhexyl polymethacrylamide
- N-di(2-ethylhexyl) polymethacrylamide
- 55 N-decylpolymethacrylamide
- N-dodecylpolymethacrylamide
- N-hexadecylpolymethacrylamide
- N-eicosanylpolymethacrylamide
- N-ethyl-N-octylpolymethacrylamide
- 60 N-methyl-N-octadecylpolymethacrylamide
- N-propyl-N-octadecenylpolymethacrylamide
- N-2-ethylhexylpolyethylacrylamide
- N-octadecyl polyethylacrylamide
- N-octadecenyl polyethylacrylamide
- 65 N-2-ethylhexylpolyacrylamide
- N-octadecylpolyacrylamide
- N-hexadecylpolyacrylamide
- N-ethyl-N-octadecyl polyacrylamide
- N-hexyl-N (ω-carboxy) undecyl polymethacrylamide
- 70 N-(b-dodecylthio) ethyl polymethacrylamide
- N-(b-octylthio) ethyl polyacrylamide
- N-(b-decyloxy) ethyl polyethylacrylamide
- N-(b-amylthio) ethyl polymethacrylamide
- 75 N-(b-isoamylthio) ethyl polypropylacrylamide

It will be apparent from all of the above that, by my invention, I have provided hydrocarbon oils which have been improved in a number of their properties and which have many uses, such as in the lubrication of internal combustion engines, for bearings subjected to high speeds and pressures, for the lubrication of gears of the hypoid, spiral and bevel types, for railroad rolling stock, for marine engines and for protective coatings on metallic surfaces subject to corrosion.

I claim:

1. A hydrocarbon oil having incorporated therein a small proportion, at least 0.01%, of an oil-soluble polymeric N-aliphatic acrylamide having a molecular weight of at least 1000 in which the aliphatic group contains an open chain of at least 8 atoms of which not more than 2 are interrupting atoms of the class consisting of oxygen and sulfur and the rest are carbon atoms.

2. A hydrocarbon oil having incorporated therein a small proportion, at least 0.01% of an oil-soluble polymeric N-aliphatic acrylamide having a molecular weight of at least 1000 in which the aliphatic group contains an open chain of at least 8 carbon atoms.

3. A hydrocarbon oil having incorporated therein a small proportion, at least 0.01%, of an oil-soluble polymeric N-aliphatic acrylamide having a molecular weight of at least 1000 in which the aliphatic group is an open chain hydrocarbon group containing at least 8 carbon atoms in the chain.

4. A hydrocarbon oil having incorporated therein a small proportion, at least 0.01%, of an oil-soluble polymeric N-alkyl acrylamide having a molecular weight of at least 1000 in which the alkyl group contains an open chain of at least 8 carbon atoms.

5. A hydrocarbon oil having incorporated therein a small proportion, at least 0.01%, of an oil-soluble polymeric N-octadecyl acrylamide having a molecular weight of at least 1000.

6. A hydrocarbon oil having incorporated therein a small proportion, at least 0.01%, of an oil-soluble polymeric N-octadecyl methacrylamide having a molecular weight of at least 1000.

7. A hydrocarbon oil having incorporated therein a small proportion, at least 0.01%, of an oil-soluble polymeric N-aliphatic acrylamide having a molecular weight of at least 1000 which is the reaction product of a polymeric acrylic acid ester and an aliphatic amine containing an open chain of at least 8 atoms of which not more than 2 are interrupting atoms of the class consisting of oxygen and sulfur and the rest are carbon atoms.

8. A hydrocarbon oil having incorporated there-

in a small proportion, at least 0.01%, of an oil-soluble polymeric N-aliphatic acrylamide having a molecular weight of at least 1000 which is the reaction product of a polymeric acrylic acid ester and an aliphatic amine which, except for the amino N atom, consists of carbon and hydrogen and contains an open chain of at least 8 carbon atoms.

9. A hydrocarbon oil having incorporated therein a small proportion, at least 0.01%, of an oil-soluble polymeric N-alkyl acrylamide having a molecular weight of at least 1000 which is the reaction product of a polymeric acrylic acid ester and an alkyl amine containing an open chain of at least 8 carbon atoms.

10. A hydrocarbon oil having incorporated therein a small proportion, at least 0.01%, of an oil-soluble polymeric N-octadecyl acrylamide having a molecular weight of at least 1000 which is the reaction product of a polymeric acrylic acid ester and octadecylamine.

11. A hydrocarbon oil having incorporated therein a small proportion, at least 0.01%, of an oil-soluble polymeric N-aliphatic acrylamide having a molecular weight of at least 1000 which is the reaction product of a polymeric methacrylic acid ester and an aliphatic amine containing an open chain of at least 8 atoms of which not more than 2 are interrupting atoms of the class consisting of oxygen and sulfur and the rest are carbon atoms.

12. A hydrocarbon oil having incorporated therein a small proportion, at least 0.01%, of an oil-soluble polymeric N-aliphatic acrylamide having a molecular weight of at least 1000 which is the reaction product of a polymeric methacrylic acid ester and an aliphatic amine which, except for the amino N atom, consists of carbon and hydrogen and contains an open chain of at least 8 carbon atoms.

13. A hydrocarbon oil having incorporated therein a small proportion, at least 0.01%, of an oil-soluble polymeric N-aliphatic acrylamide having a molecular weight of at least 1000 which is the reaction product of a polymeric methacrylic acid ester and a primary aliphatic amine which, except for the amino N atom, consists of carbon and hydrogen and contains an open chain of at least 8 carbon atoms.

14. A hydrocarbon oil having incorporated therein a small proportion, at least 0.01%, of an oil-soluble polymeric N-octadecyl acrylamide having a molecular weight of at least 1000 which is the reaction product of a polymeric methacrylic acid ester and octadecylamine.

MELVIN A. DIETRICH.